

# UNITED STATES PATENT OFFICE.

FREDERICK G. KEYES, OF EAST ORANGE, NEW JERSEY, ASSIGNOR TO COOPER HEWITT ELECTRIC COMPANY, OF HOBOKEN, NEW JERSEY, A CORPORATION OF NEW JERSEY.

## METHOD OF DRAWING WIRE FILAMENTS FOR INCANDESCENT ELECTRIC LAMPS.

1,293,116.

Specification of Letters Patent.

Patented Feb. 4, 1919.

No Drawing.

Application filed February 11, 1914. Serial No. 818,008.

To all whom it may concern:

Be it known that I, FREDERICK G. KEYES, a citizen of the United States, and resident of East Orange, county of Essex, State of New Jersey, have invented certain new and useful Improvements in Methods of Drawing Wire Filaments for Incandescent Electric Lamps, of which the following is a specification.

- 10 The present method of obtaining metallic tungsten consists in adding to tungsten tri-  
oxid ( $WO_3$ ) a suitable binding material, and then reducing in an atmosphere of hydrogen at a high temperature. The ingot thus pro-  
15 duced consists of metallic tungsten cemented together by a binding material and the next step in the process is that of subjecting the ingot to a swaging process which is also carried out at a high temperature. The swag-  
20 ing is continued until the ingot is reduced to a diameter that permits of its being drawn while hot through suitable dies until the desired sizes are obtained. The binding material is so selected as to toughen the result-  
25 ing wire.

It is a disadvantage appertaining to this process that the dies are lubricated with graphite. It is a matter of common knowledge that tungsten has a great avidity for carbon, where as it would be an advantage to prevent, if possible, any cementation. This is done in the present method of obtaining tungsten and the result is that the tungsten wire used in tungsten lamps is in reality not a pure metal, but a mixture, chemical or otherwise, of binding material and carbid.

- 30 Experience shows that a pure metal is very much more ductile than any of its alloys.  
40 The object of the present invention is to provide means for obtaining pure metallic tungsten in distinction from tungsten-tungsten carbid.

To accomplish this I dissolve tungsten tri-  
45 oxid in boric acid at  $1200^{\circ}$  to  $1400^{\circ}$  C. and electrolyze the solution thus formed. While it is impossible to electrolyze tungsten from an aqueous solution, it is readily possible to secure a deposit of pure metallic tungsten 50 from a boric acid solution at the tempera-  
tures mentioned above. The tungsten can be deposited electrolytically upon a fine tungsten wire and when a sufficient amount has

been deposited, it may be subjected to a drawing process such as is now used, or, 55 preferably, it may, in the early stages of the drawing, be drawn through dies of a special tungsten-iron-carbon alloy. Such alloys are already known in the arts and tools made of it hold their edge at a red heat. The pure 60 tungsten having, as stated, a superior quality of ductility when obtained by my process may be drawn through these special dies, thus avoiding the expensive diamond dies. As a lubricating material powdered talcum 65 may be substituted for the deleterious graphite.

I claim as my invention:

1. The method, which consists in depositing tungsten from an electrolytic bath of 70 tungsten compound in an ionizing medium upon a fine tungsten wire, and subjecting the resulting wire to a hot drawing process.

2. The method, which consists in depositing tungsten from an electrolytic bath of 75 tungsten compound in an ionizing medium upon a tungsten core, and subjecting the resulting material to a hot drawing process.

3. The method of producing ductile tungsten wire, which consists in forming a body 80 of tungsten, depositing pure metallic tungsten on said body as a core from an electrolytic bath of tungsten compound in an ionizing medium, and hot drawing the resulting material.

4. The method of producing ductile tungsten wire which consists in forming the linear body of tungsten, depositing pure metallic tungsten electrolytically upon said linear body hot drawing the resulting material with the use of a lubricating material of powdered talcum.

5. The method which consists in forming the linear body of tungsten, depositing pure metallic tungsten thereon electrolytically hot 95 drawing the resulting material through dies of tungsten iron carbon alloy with the use of a lubricating material of powdered talcum.

Signed at New York in the county of New 100 York and State of New York this 10th day of February, A. D. 1914.

FREDERICK G. KEYES.

Witnesses:

W. H. CAPEL,  
THOS. H. BROWN.